

## UNITED STATES PATENT OFFICE.

KARL J. JACOBI, OF ROSELLE, NEW JERSEY, ASSIGNOR TO PACIFIC COAST BORAX COMPANY, OF NEW YORK, N. Y., A CORPORATION OF NEVADA.

## HEAT TREATMENT OF ALLOYS.

No Drawing.

Application filed June 9, 1926. Serial No. 114,807.

This invention relates to improvements in the tempering or heat treatment of alloy steels and particularly of high speed tool steels or of high speed tools made of alloy 5 steels.

According to the present invention, the tempering or heat treatment of the tools, etc. is effected in a fused bath of a borate which is substantially neutral in reaction, such as 10 calcium borate. Such a bath, e. g. of calcium borate is neutral in the sense that it does not attack the alloy steel in an objectionable way, as does a bath of borax.

In the practice of the invention, two baths 15 may advantageously be used, the first a pre-heating bath and the second the main tempering or heat treatment bath. For example, a preheating bath of calcium bi-borate  $\text{CaB}_4\text{O}_7$  may be used for bringing the temperature of the high speed tools up to around 1800° F. and the main bath may be maintained at a temperature, e. g. around 2250° F. and the tools, after having been heated in the preheating bath to approximately the 25 temperature of that bath can then be transferred to the main bath and kept therein for a sufficient period of time to complete the heat treating operation. With the baths at a constant temperature, it can readily be 30 determined how long it takes to bring the tools to the temperature of the bath and they can thereafter be kept in the bath for a limited time, e. g. a period of around 9 to 10 minutes in the preheating bath, and about 35 3 minutes in the hardening bath after which they may be removed and put in a cooling bath at a lower temperature, e. g. at a temperature around 1000° F.

The cooling bath into which the tools are 40 placed, may advantageously be a bath containing sodium carbonate. The calcium bo-

rate remains on the tools when removed from the bath, in the form of a thin film, but by dipping the tempered or heat treated tools in a bath containing sodium carbonate, e. g. at 1000° F., this film of calcium borate will be removed at the same time that the tool is cooled to the temperature of this bath. The tools can then be further cooled or quenched by plunging them in an oil 50 bath.

Instead of using calcium borate, other stable neutral borates, such as other alkali earth borates, can be similarly used.

The temperature of the tempering or heat 55 treatment can be varied with different alloy steels, or with different tools, and the invention is not limited to the specific example given above.

## I claim:

1. The method of heat treating alloy steels which comprises subjecting them to a fused bath of an alkali earth borate.

2. The method of heat treating alloy steels which comprises subjecting them to a fused 65 bath of calcium bi-borate.

3. The method of removing a film of an alkali earth borate remaining on an article after treatment according to claim 1, which consists in immersing the article containing 70 the film in a bath containing sodium carbonate, said bath being at a temperature of about 1000° F.

4. The method of removing a calcium bi-borate film remaining on an article after 75 treatment according to claim 2, which consists in immersing the article containing the film in a bath containing sodium carbonate, said bath being at a temperature of about 1000° F.

In testimony whereof I affix my signature.  
KARL J. JACOBI.

60

65

65

80